

June 10, 1924.

1,497,421

M. M. WILCOX

TAPPET

Filed April 18, 1921



Fig. 1



Fig. 2

Gerrill M. Wilcox  
INVENTOR

By  
Gerrill M. Wilcox  
ATTORNEY

Patented June 10, 1924.

1,497,421

# UNITED STATES PATENT OFFICE.

MERRILL M. WILCOX, OF SAGINAW, MICHIGAN.

## TAPPET.

Application filed April 18, 1921. Serial No. 462,424.

*To all whom it may concern:*

Be it known that I, MERRILL M. WILCOX, a citizen of the United States, residing at Saginaw, in the county of Saginaw and 5 State of Michigan, have invented certain new and useful Improvements in Tappets; and I do hereby declare the following to be a full, clear, and exact description of the invention, such as will enable others skilled 10 in the art to which it appertains to make and use the same.

This invention relates to cam followers or tappets for use in internal combustion engines and the like and the improvement 15 pertains more particularly to a new tappet construction whereby the objects of my invention are attained.

These objects are, first, to provide a tappet that is light in weight, yet exceedingly 20 strong to resist the strains brought upon it in use and capable of being manufactured by the employment of a minimum number of operations.

A further object is to provide a tappet 25 head made of material that is inexpensive and yet admirably adapted to withstand the rapidly repeated impacts of the valve cam.

With these and certain other objects in view which will appear later in the specifications, my invention comprises the devices 30 herein described and claimed and the equivalents thereof.

In the drawings, Fig. 1 is a vertical section through a tappet embodying one form 35 of my improvement.

Fig. 2 is a similar section through a modified form of my improved tappet.

In the drawings, 1 is the tubular body or 40 shell of the tappet. 2 is the head that receives the impact of the engine cam, not shown. The end 3 of the head may be flanged as shown, if desired, and the head is provided with an axially extending cylindrical shank 4 adapted to be received in the 45 end of the tubular body and to project into it a sufficient distance to form an interior reinforcement for the tubular body 1, to prevent buckling or distortion of the body when the tappet is in action and is being rapidly reciprocated in the sliding bearing 50 or guide in which a tappet is customarily mounted in an engine.

It has heretofore been common in the design and manufacture of tappets for high 55 speed engines to make the tappet of a single piece of metal; or of two pieces, as a tubular

body and a head; or sometimes of three pieces, as a tubular body, a plug at one end and a head at the other end.

The purpose of the two-piece and three-piece tappets has been to enable the head to be made of alloy steel which is capable of being given a great degree of hardness, while the tubular body is made of softer and cheaper material.

Such multiple-piece tappets have required more operations for their manufacture and are in general more expensive to make than the one-piece tappet, but on account of the 60 advantage of lightness and because the design permits the heads to be made of alloy steel and case-hardened, the multiple-piece 65 type of tappet has come into extensive use.

I have found however, in practice, that the alloy head has serious disadvantages in 70 that it requires several incidental mechanical operations in its manufacture, thereby increasing its cost. I have also found by experience that the alloy steel heads have 75 inherent disadvantages that detract from 80 their usefulness and reduce the period of working life of the tappet.

For example, an alloy steel head must be case-hardened on its working face and then ground to exact size. The case-hardening or 85 carbonizing process, as is well known, consists in first electroplating the alloy steel head with copper, then grinding off the copper from the face of the head and then carbonizing the head in the furnace, the copper plating preventing the absorption of carbon by the surfaces that need not necessarily be hardened, namely, all surfaces except the working face.

The head after hardening requires to be 90 ground to its final shape, inserted in the tubular body and then spot-welded. The foregoing operations, while necessary in the construction of an alloy steel head tappet, 95 are expensive.

In the commercial production of hardened alloy steel tappets the face of the head is made extremely hard, but only for a short depth, and in the oil-quenching step of the hardening process there apparently is left 100 sufficient heat in the body of the head to result in slightly annealing that part of the metal of the head which lies directly back of the thin hard steel face.

Since alloy steel is intended for and particularly adapted to service requiring high 105 tensile strength, and is not so well adapted

to resist impact, it follows in practice that the constant hammering of the cam against the tappet produces a multitude of microscopic surface checks and imperfections in the thin hardened face. It is possible that this condition is aggravated by the shrinkage strains which are set up in the hardened surface when the heated metal of the body of the head cools subsequent to the initial chilling of the face, resulting in the minute temperature cracks on the surface. In any event, it has been proven that case-hardened alloy steel tappet heads are not sufficiently durable in practice to warrant the high expense that must be put into their manufacture.

To overcome these defects, while still preserving the general design, lightness and strength of multiple-piece tappets, I have devised the improvement herein illustrated.

I have discovered that a grey iron casting, which may preferably be chilled, and then ground, fitted and secured to the tubular body by welding produces a tappet head that is admirably adapted to withstand the impacts of the cam, that has a face which has no surface checks or cracks and which tends to become more dense with continued use, instead of developing cracks, as is the case with the hardened alloy heads previously referred to, and it also eliminates the necessity for employing the preliminary steps heretofore required for machining, electroplating and case-hardening; steps which constitute a considerable part of the entire cost of manufacturing tubular tappets.

In carrying out my invention in accordance with the construction of Fig. 2, I first make a tappet head of cast iron, grind the shank of the head to size, insert the shank in the tubular body and spot weld the tubular body to the shank as indicated at 5, Fig. 2 and then grind the exterior of the tubular body and the face of the head to finished dimensions.

The working face of a ferrous casting so prepared is almost perfectly smooth, highly polished and in use becomes glass hard without indentations. There are no apparent surface checks or tension strains and the material becomes more and more dense with continued use under the hammering action of the engine cams.

There is no difficulty in spot welding the

thin metal tappet 1 to the shank 2, a commercially perfect welded union being attained by the use of the ordinary spot welding machine.

In the type of tappet shown in Fig. 2, the tubular body 1 is made of a separate piece of metal, which may be cold rolled steel, or its equivalent, but the tappet may be made as shown in Fig. 1, where the entire tappet, including the head, is cast in one piece, the head may be cast in a chill and the tubular body being preferably cast in sand according to the methods of procedure which are well known in foundry practice.

By making the tappet head of either common grey iron or of chilled iron instead of alloy steel I have not only improved the wearing qualities of the tappet surface, but have reduced the cost of manufacture to a small part of the cost of a tubular tappet having a case-hardened head formed of alloy steel or similar material.

Having thus described my invention, what I claim and desire to secure by Letters Patent is:

1. As a new article of manufacture, a tappet comprising a hollow tubular stem and a head formed of a chilled iron casting, said head and stem cast integral.

2. As a new article of manufacture, a tappet comprising a cast iron stem and a head formed of a chilled iron casting, said head and stem formed integral, for the purposes set forth.

3. As a new article of manufacture, a tappet formed of cast iron and having its cam-engaging face of chilled metal.

4. As a new article of manufacture, a tappet formed of cast iron and having a discous head formed with a cam-engaging face and also having a stem, said head portion being of chilled metal at and adjacent its cam-engaging face.

5. As a new article of manufacture, a tappet formed of cast iron and having a discous head portion formed with a cam-engaging face and also having an integral stem portion, said head portion being of chilled metal at and adjacent its cam-engaging face and the remainder of said tappet being unchilled.

In testimony whereof, I affix my signature.

MERRILL M. WILCOX.